

# UNITED STATES PATENT OFFICE.

ELTWEED POMEROY, OF NEWARK, NEW JERSEY, ASSIGNOR TO THE  
POMEROY DUPLICATOR COMPANY, OF NEW JERSEY.

## STENCIL-PLATE.

SPECIFICATION forming part of Letters Patent No. 601,479, dated March 29, 1898.

Application filed March 16, 1896. Serial No. 583,455. (No model.)

*To all whom it may concern:*

Be it known that I, ELTWEED POMEROY, a citizen of the United States, residing at Newark, in the county of Essex and State of New Jersey, have invented a certain new and useful Improvement in Stencil-Plates, of which the following is a specification.

My invention relates to that class of stencil-plates which comprise a base of an open veil-like material, preferably of paper, an example of which is the well-known Japanese paper called "yoshino" in Japan and "dental paper" in this country, which base is provided with a coating of such a nature as to be readily removable by the pressure of the writing implement from the openings of the base without destroying, when written upon with ordinary care, the threads or fibers crossing the line of writing to such an extent as to cut out the centers of loop letters.

More particularly my invention relates to the coating for such stencil-plates, and it depends upon the discovery that by treating pure paraffin by heat in a vessel closed except for a small vent the nature of the paraffin will be altered and what I may term its "toughness" be altered, as well as its melting-point lowered.

In carrying out my invention I take, for example, fifteen pounds of paraffin having a high melting-point—as, for instance, 135° or 140° Fahrenheit—and place the same in a closed vessel having a small tube or vent extending from its top. The contents of the vessel are then treated for from an hour and a half to four hours, according to the intensity of the fire beneath. The paraffin appears to boil vigorously and throw off fumes and vapors, and I have found that generally a small explosion occurs shortly after the paraffin is heated. For this reason I prefer and recommend that the operation be

carried on in the open air. To determine when the operation has been carried sufficiently far, a small quantity of the paraffin is poured from the vessel and its melting-point taken. If the melting-point has been lowered one or two degrees, the treatment is considered finished. After one has had some experience in performing this operation the point where treatment is carried sufficiently far can be determined by the appearance and color of the boiling paraffin. The product differs in its structure from the original paraffin treated in that it is less coherent or more friable and more oily. It also does not have as clear a color.

A base such as yoshino-paper coated with this coating will be found to work as a stencil-plate in a very superior manner to pure paraffin of the original melting-point of the coating, giving a stencil in which the liability of cutting out the centers of loop letters is almost if not entirely eliminated.

I claim—

1. A stencil-plate having a base substantially as described, and having a coating substantially as described, consisting of a hydrocarbon formed by heating paraffin, which hydrocarbon is characterized by greater friability than paraffin.

2. A coating for stencil-plates consisting of a hydrocarbon formed by heating paraffin, which hydrocarbon is characterized by a reduction in consistency, toughness and melting-point from paraffin, substantially as described.

This specification signed and witnessed this 9th day of March, 1896.

ELTWEED POMEROY.

Witnesses:

EUGENE CONRAN,  
JOHN R. TAYLOR.